

June 5, 1928.

1,672,821

C. MARTELL

SUBMARINE CABLE CORE AND INSULATION THEREFOR

Filed Oct. 7, 1924

*Fig. 1.*



*Fig. 2.*



Inventor  
Charles Martell  
by Heaton, Atty.

## UNITED STATES PATENT OFFICE.

CHARLES MARTELL, OF CICERO, ILLINOIS, ASSIGNOR TO WESTERN ELECTRIC COMPANY, INCORPORATED, OF NEW YORK, N. Y., A CORPORATION OF NEW YORK.

## SUBMARINE CABLE CORE AND INSULATION THEREFOR.

Application filed October 7, 1924. Serial No. 742,142.

This invention relates to an improved submarine cable core, particularly of the continuously loaded type, and an improved insulation for such cores.

5 The materials usually employed for insulating deep sea cables are gutta-percha and balata. Gutta-percha is to be preferred to balata for durability and long life. It oxidizes very slowly, is substantially non-water 10 absorbent, and as a result will last for a very long length of time. Balata oxidizes more rapidly and its useful life as an insulation is considerably less than that of gutta-percha. Balata, however, has better electrical 15 characteristics than gutta-percha, and electrical impulses can be transmitted more quickly through a conductor insulated with balata than through a conductor insulated with gutta-percha. Submarine cable insulation is often made from a mixture giving better electrical characteristics than gutta-percha and at the same time greater durability than balata. Hence, durability is sacrificed to obtain better electrical characteristics. 20 Moreover, the price of gutta-percha is considerably higher than that of other types of insulation materials. Other so-called gum exudates of the same grade are in general much less expensive than gutta-percha. It is, therefore, desirable from a cost standpoint to utilize wherever possible cheaper grades of plastic insulating materials.

An object of the invention is to produce 35 an improved submarine cable core.

Another object is to produce an inexpensive, durable and efficient insulation for electrical conductors.

The invention comprises an insulation 40 consisting of alternate laminations of gutta-percha and a plastic material having better electrical characteristics, and in its preferred form two laminations of gutta-percha and one lamination of balata, one layer of the 45 gutta-percha being adjacent to the conductor, and the other forming the outside shell of the insulation with the layer of balata lying between the two layers of gutta-percha.

50 In the attached drawings,

Fig. 1 is a fragmentary side elevation of submarine cable core, embodying the invention, and

Fig. 2 is a cross-section taken on the line 2-2 of Fig. 1.

Referring to the drawings, the improved submarine cable core comprises a copper conductor consisting of a central portion 9 and a plurality of tapes 10, and spiralled thereon a loading material 11, which may 60 consist of the material known as permalloy, the metallurgical constitution and electrical characteristics of which are set forth in the patent to G. W. Elmen, No. 1,586,884, issued June 1, 1926. Adjacent to the loading material 11 and entirely surrounding it is a 65 layer of gutta-percha 12, and surrounding the layer of gutta-percha 12 is a layer of balata 13. Adjacent to the balata 13 and comprising the outer shell of insulation is 70 another layer of gutta-percha 14.

The invention as embodied in the drawings may take a variety of forms. For instance, the number of laminations need not be limited to three, but may be any number 75 which might be required, depending upon the conditions or circumstances in which the core is to be used. It is desirable, however, to have a layer of gutta-percha next to the conductor because of a slight acid content 80 in balata which may in time cause a corrosion of the metallic conductor or loading material as the case may be. It is also desirable on account of the physical properties of gutta-percha that the outside layer or lamination be of that substance. In the preferred form of the invention the layers of 85 gutta-percha are made no thicker than is required to insure durability, the balance of the insulation being balata. In a desirable 90 composite insulation of this preferred type the two layers of gutta-percha taken together are of about the same thickness as the single layer of balata interposed between them.

The advantage of this type of insulation 95 over insulations which have heretofore been used is that the desirable characteristics of both the gutta-percha and balata are utilized. It is well-known that balata has better electrical characteristics than gutta-percha. For instance its conductance, which is proportioned by the total power losses in the dielectric, is lower. An insulation of gutta-percha and balata produced according to 100 105 this invention and in which the proportion

of the two materials is about equal, has a conductance at 24° C. of about 6 micromhos per nautical mile at 900 cycles; while an insulation of pure gutta-percha has a conductance of from 20 to 50 micromhos per nautical mile under the same conditions.

Gutta-percha, however, on account of its longer life, is to be preferred to balata for economical purposes. As an example, a submarine cable in which the conductor is insulated exclusively with balata would in a relatively shorter time than in the case of gutta-percha be unfit for use because the balata would deteriorate, principally by oxidation, and the acid in the balata would corrode the conductor. This would cause a very great retardation in the speed at which messages could be transmitted from end to end of the cable and would ultimately cause a breaking down of the entire cable.

The price of balata, however, is comparatively low, a satisfactory grade of gutta-percha as a general rule being at times as much as two or even three times as high. The lack of economy in the use of pure balata for insulation as mentioned above, is due to the shorter life of such material as compared to gutta-percha, due to its more rapid disintegration. The initial cost is low, and by means of the present invention the low initial cost of balata is taken advantage of, and decomposition or deterioration of the balata avoided by means of protective layers of gutta-percha as herein disclosed.

It is not absolutely necessary that balata be used as one of the materials which will go to make up an insulation produced according to this invention. Any material which has better electrical characteristics than gutta-percha may be employed. Furthermore, if it is desirable to lower the cost of the insulation where the electrical requirements are not so exacting, a material having no better electrical characteristics than gutta-percha but which is cheaper in price may be employed instead of the balata. However, from the standpoint of all-around

adaptability, balata is to be preferred for use in this manner.

What is claimed is:

1. An insulation for electrical conductors comprising a layer of balata, and a layer of gutta-percha.

2. An insulation for electrical conductors comprising a layer of balata, and a layer of gutta-percha, the layer of balata being thicker than the layer of gutta-percha.

3. An insulation for electrical conductors comprising a plurality of layers of balata and gutta-percha, and so arranged that the desirable characteristics of each material is utilized.

4. An insulation for electrical conductors comprising alternate layers of balata and gutta-percha.

5. An insulation for electrical conductors comprising a layer of balata positioned between two layers of gutta-percha.

6. A submarine cable comprising a conductor, and an insulation consisting of a thick layer of balata interposed between relatively thin layers of gutta-percha.

7. A submarine cable comprising a conductor, a magnetic loading material associated therewith, and an insulation consisting of alternate layers of gutta-percha and balata.

8. A submarine cable comprising a conductor, a magnetic loading material associated therewith, and an insulation consisting of a thick layer of balata interposed between relatively thin layers of gutta-percha.

9. An insulation for electrical conductors comprising a plurality of layers of gutta percha and balata and so arranged that the gutta percha is in contact with the conductor and also constitutes the outer sheath of the insulation.

In witness whereof, I hereunto subscribe my name this 18th day of September, A. D. 1924.

CHARLES MARTELL.